

1

3,089,759

## CONCENTRATION OF RARE EARTHS

Hugh J. Bronaugh, Chattanooga, and Paul R. Kruesi, Signal Mountain, Tenn., assignors, by mesne assignments, to Vitro Corporation of America, New York, N.Y., a corporation of Delaware  
No Drawing. Filed Apr. 18, 1960, Ser. No. 22,661  
7 Claims. (Cl. 23—296)

The present invention relates to the concentration of rare earth elements. More particularly it relates to the concentration of europium.

The usefulness of europium as a neutron absorbing material in the field of nuclear power has greatly increased the importance of this rare earth metal. It may be recovered by known and proven methods, such as the reduction of the tervalent ion to the divalent state and subsequent precipitation of europous sulfate, but this requires a feed material that has been previously enriched in europium to a value greater than that normally present in the ore. As the concentration of europium increases, a corresponding increase in recovery is obtained.

Although the classical methods of obtaining europium concentrates for subsequent recovery of europium tend to produce a fraction containing a higher concentration than the present procedure, these methods are laborious and time consuming. Good recoveries can be obtained according to the present invention with a concentrate containing a europium oxide to total oxide ratio of as little as 0.2%.

It is thus an object of the present invention to provide a simple, effective and speedy process for concentrating rare earth elements and particularly europium.

Another object is to obtain good recoveries of europium from a concentrate containing as little as 0.2% europium oxide.

These and other objects of the present invention will become apparent as the description proceeds.

In principle the present invention comprises heating a solution of rare earth chlorides at a temperature from about 190° F. to about 203° F. until a specific gravity of about 1.85 to about 1.92 is achieved, and then cooling the solution to a temperature of from about 149° F. to about 160° F. during a period of about 1 to about 3 hours to cause crystallization of the desired rare earth elements. According to such a process the rare earths with atomic numbers greater than 59, but including yttrium, are enriched in the crystals whereas, the lighter rare earths, lanthanum and cerium are concentrated in the mother liquor. The concentrated europium is then recovered from the crystals by known methods.

The mixed rare earth chlorides which are the starting material for the present process may be obtained by treating the mineral monazite, which consists predominantly of rare earth phosphates, with sodium hydroxide to form the rare earth hydroxides and then dissolving the latter compounds in hydrochloric acid. The mixed rare earth chloride crystals are then obtained by removing water from a dilute chloride solution containing rare earth cations until crystallization takes place.

The present process depends on the discovery that, contrary to expectations, the heavier rare earth elements are separated by selective crystallization on heating followed by rapid cooling. It is believed that this separation is due to the formation of an unstable crystalline hydrate. It is necessary, however, that the crystals be separated immediately; otherwise on standing, an equilibrium will be attained resulting in an ineffective separation.

The present process is applicable, as previously described, to solutions of mixed rare earth chlorides pro-

2

duced as indicated herein, from monazite. It is equally applicable to the concentration of heavier rare earth metals from solutions of mixed rare earth cations which have previously been treated as described in copending patent application Serial No. 22,660, filed on even date herewith by Paul R. Kruesi, now United States patent number 3,089,758, and entitled "Concentration of Rare Earths." According to said copending application, the mixed rare earth chlorides are first treated to obtain crystals enriched in the lighter rare earths, lanthanum, cerium and praseodymium. This is followed by a treatment to produce crystals enriched in the heavier rare earth metals. The mother liquor from this second treatment is then processed according to the method described herein to yield a crop of crystals further enriched in the heavier rare earth metals. These enriched crystals may in turn be dissolved in water and circulated through a bed of metallic zinc to reduce the europic ion to the europous ion. The addition of ammonium sulfate and barium ion to the solution containing the europous ions precipitates europous sulfate in a matrix of barium sulfate. The latter material may then be processed according to the method described in copending patent application Serial No. 22,834, filed on even date herewith by Hugh J. Bronaugh, and entitled "Purification of Europium," to yield europium oxide having a purity of about 99.8% to 99.9%.

The following examples serve to illustrate the present invention without, however, limiting the same thereto.

## EXAMPLE 1

Rare earth chloride crystals weighing 1,000 pounds were dissolved in approximately 80 gallons of water in a steam-jacketed, glass-lined vessel. The solution was evaporated at a temperature of 194° F. until the specific gravity reached 1.92. The solution was then cooled to 154° F. during a specific time period of 1.5 hours. The crystals thus obtained were separated from the mother liquor by centrifugation.

The total rare earth content of the starting material was found to be 45.5%, calculated as oxides. The ratio of cerium, calculated as CeO<sub>2</sub>, to total oxide was 36%. The ratio of europium, calculated as Eu<sub>2</sub>O<sub>3</sub>, to total oxide was 0.20%.

The product weighed 448 lbs. and had a total oxide content of 45.4%, of which the ratio of CeO<sub>2</sub>, to total oxide was 26.6% and the ratio of Eu<sub>2</sub>O<sub>3</sub>, to total oxide was 0.34%.

The europium content of the starting material was 50 (1000) (0.455) (0.002)=0.91 lb. while that of the product was (448) (0.454) (0.0034)=0.695 lb. Thus the percent recovery was

$$\frac{0.695}{0.91} \times 100 = 76.3\%$$

## EXAMPLE 2

1,092 lbs. of rare earth chloride crystals having a total oxide content of 45.5%, of which the cerium content, calculated as CeO<sub>2</sub> was 36.2%, and of which the europium content calculated as Eu<sub>2</sub>O<sub>3</sub>, was .21%, were treated at a temperature of 199° F. until the specific gravity was 1.90. They were then cooled to 151° F. for a period of about 2 hours. The separated crystals, weighing 480 lbs. had a total oxide content of 45.9%, of which the cerium content, as CeO<sub>2</sub>, was 28.2% and of which the europium content, as Eu<sub>2</sub>O<sub>3</sub>, was 0.32%. Eu<sub>2</sub>O<sub>3</sub> in feed=1.04 lbs.; Eu<sub>2</sub>O<sub>3</sub> in product=0.71 lb.; percent recovery=68%.

A study of the cerium oxide to total oxide ratio in each of the cited examples will reveal that the product crystals are depleted in cerium. Thus the concentra-

tion of cerium has been increased in the mother liquor. Data obtained from several laboratory experiments set forth in the following table show the enrichment of various rare earth metals in the product crystals or the mother liquor which is accomplished according to the present process.

at completion of the experiment is equal to the volume present in the crystallizer body at the start of the experiment.

(2) The composition of the solution left in the crystallizer body at the completion of the experiment is equal to the composition of the solution present in the crys-

ANALYSIS (WT. PERCENT  $R_2O_3$ )

|                    | Y   | La | Pr  | Nd | Sm  | Eu   | Gd  | Tb   | Dy  | Ho   | Er   |
|--------------------|-----|----|-----|----|-----|------|-----|------|-----|------|------|
| Feed-----          | 5   | 40 | 9.6 | 29 | 6.1 | 0.22 | 4.1 | 0.4  | 2.3 | 0.2  | 0.25 |
| 50% Split:         |     |    |     |    |     |      |     |      |     |      |      |
| Mother Liquor----- | 4.4 | 50 | 9   | 26 | 3.0 | 0.08 | 2.1 | 0.23 | 1.2 | 0.11 | 0.2  |
| Crystals-----      | 5.5 | 27 | 10  | 40 | 8.7 | 0.3  | 6.5 | 0.6  | 3.0 | 0.25 | 0.3  |

## EXAMPLE 3

This example shows the application of the present process to a rare earth mixture which has previously been treated according to the process described in the aforementioned copending application Serial No. 22,660.

The crystallizer was operated continuously, twenty-four (24) hours a day for a ten (10) day period. A complete cycle, that is, three (3) crystallizations, was performed each day. A typical procedure for one cycle is described as follows:

## CONCENTRATION OF RARE EARTHS

- (1) Feed 1500 gallons of rare earth chloride solution to the crystallizer.
- (2) Concentrate solution by vacuum distillation at 160° F. until a specific gravity of 1.85 is obtained.
- (3) Cool the solution slowly to 123° F. during a twelve (12) hour period.
- (4) Separate cold crystals by centrifugation, returning mother liquor to crystallizer.
- (5) Concentrate the solution in the crystallizer by vacuum distillation at 160° F. until a specific gravity of 1.85 to 1.90 is obtained.
- (6) Cool the solution to 158° F. and separate the hot crystals as quickly as possible (crystals must be separated within a three (3) hour time limit). Return the mother liquor to the crystallizer.
- (7) Recrystallize the hot crystals by dissolving them in water, concentrating the solution by evaporation to a specific gravity of about 1.90 at a temperature of 195° F. Cool the mixture to 155° F. and separate the hot-hot crystals by centrifugation, returning the mother liquid to the vacuum crystallizer.

Table I presents the data collected from this ten (10) day experiment.

Table I  
CRYSTALLIZATION DATA<sup>1</sup>

|                                      | Feed   | Cold Crystals | Hot Crystals | Hot-Hot Crystals |
|--------------------------------------|--------|---------------|--------------|------------------|
| Wt. of Chloride Crystals, lbs.       | 71,523 | 26,627        | 9,699        |                  |
| Wt. of $R_2O_3$ , lbs. (Total Oxide) | 39,915 | 32,353        | 12,238       | 4,403            |
| Average Total Oxide (T.O.), percent  | 45.20  | 45.95         | 45.35        |                  |
| Average $CeO_2$ /T.O., percent       | 44.88  | 48.87         | 35.39        | 24.76            |
| Average $Eu_2O_3$ /T.O., percent     | 0.089  | 0.044         | 0.22         | 0.42             |

<sup>1</sup> Assumptions.

(1) The volume of solution left in the crystallizer body

## 20 Material balance:

$$\frac{32,353 + 4,403}{39,915} \times 100 = 94\%$$

## Europium balance:

- Feed: (39,915) (0.00089) = 35.5 lbs.  
Cold crystals: (32,353) (0.00044) = 14.2 lbs.  
Hot-hot crystals: (4,403) (0.0042) = 18.5 lbs.  
Yield:

$$\frac{18.5}{35.5} \times 100 = 52\%$$

## Recovery:

$$\frac{32.7}{35.5} \times 100 = 92\%$$

## Cerium balance:

- Feed: (39,915) (0.4488) = 17,900 lbs.  
Cold crystals: (32,353) (0.4887) = 15,800 lbs.  
Hot-hot crystals: (4,403) (0.2476) = 1,090 lbs.  
Yield:

$$\frac{15,800}{17,900} \times 100 = 88\%$$

## Balance:

$$\frac{16,890}{17,900} \times 100 = 94.4\%$$

As many and varied modifications of the subject matter of this invention will become apparent to those skilled in the art from the detailed description given herein, it should be understood that this invention is to be limited only in accordance with the appended claims.

## What is claimed is:

1. A process for the concentration of rare earth elements comprising heating a solution of chlorides of said elements at a temperature from about 190° F. to about 203° F. until the specific gravity is from about 1.85 to about 1.92, cooling said solution to a temperature of from about 149° F. to about 160° F. during a period of from about 1 to about 3 hours to cause crystallization of rare earth compounds with an increased content of compounds selected from the group consisting of yttrium and rare earth elements having atomic numbers greater than 59, and immediately separating the crystals from the mother liquor.
2. A process for the concentration of europium comprising heating a solution of rare earth chlorides at a temperature from about 190° F. to about 203° F. until the specific gravity is from about 1.85 to about 1.92, cooling said solution to a temperature of from about 149° F. to about 160° F. during a period of from about 1 to about 3 hours to cause crystallization of said concentrated europium, and immediately separating the crystals from the mother liquor.
3. A process according to claim 1 wherein the ratio of

europlum to total rare earths expressed as the oxides is at least about 0.2% in the starting material and at least about 0.3% in the final crystals.

4. A process according to claim 1 wherein the ratio of europlum to total rare earths expressed as the oxides is at least about 0.2% in the starting material and at least about 0.4% in the final crystals.

5. A process according to claim 2 wherein the ratio of europlum to total rare earths expressed as the oxides is about 0.2% in the starting material and about 0.3% in the final crystals.

6. A process according to claim 2 wherein the ratio of europlum to total rare earths expressed as the oxides is

about 0.2% in the starting material and about 0.4% in the final crystals.

7. A process according to claim 2 wherein the time of cooling is about 1.5 to 2 hours.

**References Cited in the file of this patent**

**UNITED STATES PATENTS**

2,013,767 Schulze ----- Sept. 10, 1935  
2,199,697 Fleck ----- May 7, 1940

**OTHER REFERENCES**

Vickery: Chem. of the Lanthanums (1953), pages 110 to 123.